# EUROPEAN PATENT SPECIFICATION

(11) **EP 0 736 120 B1**
(45) Date of publication and mention of the grant of the patent: **21.01.1998**
(21) Application number: 95907233.1
(22) Date of filing: 20.12.1994
(51) Int. Cl.: D21H 13/26

(54) **LAYERED SMOOTH SURFACE ARAMID PAPERS OF HIGH STRENGTH AND PRINTABILITY**
ARAMIDPAPIER MIT HOHER WIDERSTANDSFAEHIGKEIT UND BEDRUCKBARKEIT UND EINER GLATTEN SCHICHTENFOERMIGEN OBERFLAECHE
PAPIERS ARAMIDES A SURFACE LISSE MULTICOUCHE TRES RESISTANTS, SE CARACTERISANT PAR UNE APTITUDE ELEVEE A L'IMPRESSION

(30) Priority: 21.12.1993 US 170841
(43) Date of publication of application: 09.10.1996
(73) Proprietor: E.I. DU PONT DE NEMOURS AND COMPANY, Wilmington Delaware 19898 (US)
(72) Inventor: BURKS, Philip, Parks, Jr., Chesterfield, VA 23832 (US); HESLER, Lee, James, Richmond, VA 23235 (US)
(74) Representative: Abitz, Walter, Dr.-Ing.
(86) International application number: US9414672
(87) International publication number: WO9517549

(56) References cited:
- WO-A-94/16142
- US-A- 5 076 887
- US-A- 5 089 088

## Description

### Background of the Invention

This invention relates to an improved layered aramid paper having a smooth surface and good tensile and tear strengths. The smooth surface provides for better print clarity and makes such papers particularly useful for high temperature label applications. Prior art techniques that improve on surface smoothness often lead to a reduced level of mechanical strength and/or thermal stability. Moreover, synthetic papers which have been pressed or calendered at high temperature and pressure will generally have fibers on the surface which cause roughness or snagging when the surface of the paper is worked during end use processing.

US-A-5,076,887 describes a multi-layered, high temperature resistant pressboard. All layers have the same uniform distribution of polyaramid fibrids and floc. The surface smoothness is not sufficient for the purpose of the present invention.

US-A-5,089,088 describes flash expansion of moist multi-layered boards, wherein each layer comprises the same uniform composition comprising aramid floc bonded by aramid fibrid.

### Summary of the Invention

This invention provides a multi-layered calendered aramid paper having a surface suitable for high quality printing characterized in that the paper contains from 40 to 55% by weight of fibrids and comprises a substrate layer which consists essentially of aramid fibrids and floc and one or two surface layers, each bonded to the substrate layer to form a single consolidated sheet, said surface layer(s) comprising from 10 to 67% of the weight of the paper and consisting essentially of from 65 to 90% by weight aramid fibrids and from 10 to 35% by weight aramid floc and wherein the entire surface of the paper is calendered and the sheet has a density of from 0.8 to 1.0 g/cc and a thickness of from 1 to 30 mils (0.0254 to 0.762 mm).

### Detailed Description of the Invention

The multi-layered aramid papers of the invention are comprised of layers of different compositions to provide desired properties. The surface layer(s) provide a smooth surface and contain from 65 to 90% aramid fibrid and from 10% to 35% of aramid floc. The surface layer(s) constitutes from 10 to 67% of the weight of the paper. The substrate layer provides high tear strength. In order for the multi-layered paper to behave as a unitary structure, it is preferred that the fibrous materials at the interface between layers be intermingled. This is achieved by depositing a layer of furnish, i.e., a papermaking aqueous dispersion of floc and fibrid on an undried, previously formed layer of furnish in a paper making machine or by simultaneously depositing the layers of different composition on the screen of the paper making machine using a 2 or 3 layer hydraulic type headbox. The paper coming off the machine is dried and calendered, to a thickness of from 1 to 30 mils. The density of the layered paper is from 0.8 to 1.0 g/cc for use as labels.

It has been found that the multi-layered papers of this invention have excellent mechanical properties. The smooth surface retains a high degree of smoothness even after the necessary working to prepare it for end use applications. This quality is important if print clarity and color density is to be achieved.

Aramid floc is high temperature resistant floc or short fiber cut from longer aramid fiber, such as those prepared by processes described in U.S.-A-3,063,966; 3,133,138; 3,767,756 and 3,869,430. It refers to short fibers typically having a length of 2 to 12 mm and a linear density of 1-10 decitex, made of aromatic polyamide which is non-fusible.

The aramid fibrids can be prepared using a fibridating apparatus where a polymer solution is precipitated and sheared in a single step as described in U.S. -A-3,756,908.

### Tests and Measurements

Total Break Strength. The tensile break strength of paper is determined based on ASTM method D 828-87 for "Standard Test Method for Tensile Breaking Strength of Paper and Paperboard". Specimens are 2.54 cm wide and 20.3. cm long and the jaws of the tensile testing machine are initially separated by 12.7 cm. Ten paper samples are tested in the machine direction (MD) and ten are tested in the cross direction (CD) and the values for each direction are averaged. The total of the MD and CD strengths is divided by paper density and paper basis weight to obtain the Total Break Strength.

Thickness. Thickness of papers is determined using calipers in accordance with ASTM D 374-79 (1986).

Density. Density of papers is determined by determining the weight per unit area of the paper (Basis Weight) in accordance with ASTM D 646-86 and dividing by the thickness.

Abraded Fiber Count.

In order to further investigate the abrasion qualities of these papers, the papers were folded and the edge of the fold was viewed against a dark background. The number of fibers extending greater than about 0.5 mm above the solid paper surface was taken as the Abraded Fiber Count (per centimeter) and indicates the degree of roughness of the sample.

The following examples are illustrative of the invention and are not to be construed as limiting.

### EXAMPLES

### Example 1

A two layered structure was made by combining fibrids of poly(m-phenylene isophthalamide) prepared as described in Example 1 of U.S. Pat. No. 3,756,908 and floc prepared by dry spinning poly(m-phenylene isophthalamide) from a solution containing 67% dimethyl acetamide (DMAc), 9% calcium chloride and 4% water. The spun filaments were flooded with an aqueous liquid and contained about 100% DMAc, 45% calcium chloride and 30-100% water based on dry polymer. The filaments were washed and drawn 4X in an extraction-draw process in which the chloride and DMAc contents were reduced to about 0.10% and 0.5%, respectively. The filaments had a denier of 2 (2.2 dtex) and typical properties were: elongation to break, 34%, and tenacity, 4.3 grams/denier (3.8 dN/tex). The filaments were then cut to floc length of 0.27 inch (0.68 cm) and slurried in water to a concentration of about 0.35%.

Blends of fibrids and floc were separately fed to a 2-layer hydraulic type headbox which maintains each blend as a distinct layer until the slice exit where limited mixing of the layers occurs. This allows good bonding between the layers while still maintaining the individual nature of each layer. The formed sheet is then processed as is normally done on a fourdrinier paper machine by pressing and drying.

The papers are dried completely using infrared heaters before being calendered at 320°C at a line speed of 30 feet per minute (9 meters per minute) using a pressure of 725 pounds per linear inch (130 kg/cm).

The composition of the layers varied from 35 to 65% fibrid, the remainder being floc. The basis weight of each layer was adjusted so that the high fibrid layer (65% fibrid) ranged from 33 to 67% of the total basis weight of the final sheet. The total fibrid content of the test papers ranged from 45 to 55% of the sheet versus 53% for the single layer control papers (C1-1). Table 1 gives the basis weight of each layer and its composition.

**Table 1**

| Run Number | Total Sheet | | | Substrate Layer | | | Surface Layer | | |
|---|---|---|---|---|---|---|---|---|---|
| | BW aim g/m² | % Fibrid | % Floc | BW aim g/m² | % Fibrid | % Floc | BW aim g/m² | % Fibrid | % Floc |
| 1-1 | 42 | 45 | 55 | 28 | 35 | 65 | 14 | 65 | 35 |
| 1-2 | 42 | 50 | 50 | 21 | 35 | 65 | 21 | 65 | 35 |
| 1-3 | 42 | 55 | 45 | 14 | 35 | 65 | 28 | 65 | 35 |
| C1-1 | 42 | 53 | 47 | 42 | 53 | 47 | - | - - | |

The amount of loose fibers on the surfaces of the sheet as a result of mechanical working of the calendered paper was measured (Table 2). Side 1 is the substrate layer (low fibrid content layer) and Side 2 the surface (high fibrid content) layer.

**Table 2**

| Abraded Fiber Count | | |
|---|---|---|
| Sample Number | Fiber Count (per 5 cm) | |
| | Side 1 | Side 2 |
| 1-1 | 20 | 0 |
| 1-2 | 12 | 2 |
| 1-3 | 14 | 0 |
| C1-1 | 14 | - |

Even with the significant reduction in the number of loose fibers on the surface of the high fibrid content papers, superior mechanical properties are maintained versus a control paper of similar average composition but with no layering (Table 3).

**Table 3**

| Calendered Paper Properties | | | | |
|---|---|---|---|---|
| Sample Number | 1-1 | 1-2 | 1-3 | C1-1 |
| B.W.*, oz/yd² | 1.3 | 1.5 | 1.4 | 1.3 |
| (g/m²) | (44.1) | (50.9) | (47.5) | (44.1) |
| Thickness, mils | 2.0 | 2.5 | 2.2 | 2.4 |
| (mm) | (0.051) | (0.064) | (0.056) | (0.061) |
| Density, g/cc | 0.82 | 0.89 | 0.86 | 0.72 |
| B.S. **, lb/in MD/CD | 15/7 | 21/10 | 18/7 | 20/8 |
| (N/cm) | (26/12) | (37/18) | (32/12) | (35/14) |
| Eb***, MD/CD | 4/3 | 6/3 | 5/2 | 6/3 |
| Elmendorf Tear, g MD/CD | 108/191 | 120/193 | 87/166 | 127/215 |
| (N) | (1.06/1.87) | (1.18/1.89) | (0.85/1.63) | (1.25/2.11) |
| Shrinkage @ 300°C, % MD/CD | 2/0 | 2/0 | 2/0 | 2/0 |

| | | | | |
|---|---|---|---|---|
| * Basis Weight | | | | |
| ** Break Strength | | | | |
| *** Break Elongation | | | | |

### Example 2

Layered structures, 4.0-4.5 oz/yd² (135.6-152.6 g/m²) were produced with high fibrid layers on both top and bottom of the structure. The top and bottom plies (outer layers) had equal basis weight. The top and bottom layers contain 65% fibrid and 35% floc. The top layer was applied using a secondary headbox jetting the furnish onto an already formed sheet which was prepared using the headbox of Example 1. The control (C2-1) was a single layer paper.

**Table 4**

| Run Number | Total Sheet | | | Each Outer Layer | | | Inner (Substrate) Layer | | |
|---|---|---|---|---|---|---|---|---|---|
| | BW aim g/m² | % Fibrid | % Floc | BW aim g/m² | % Fibrid | % Floc | BW aim g/m² | % Fibrid | % Floc |
| 2-1 | 132 | 46 | 54 | 24 | 65 | 35 | 84 | 35 | 65 |
| 2-2 | 132 | 55 | 45 | 44 | 65 | 35 | 44 | 35 | 65 |
| C2-1 | 137 | 47 | 137 | 53 | 47 | - | - | - | - |

Improvement in the amount of loose fibers on the surface as a result of mechanical working of the paper is obvious from Table 5.

**Table 5**

| Abraded Fiber Count | |
|---|---|
| Sample Number | Fiber Count (per 5 cm) |
| 2-1 | 5 |
| 2-2 | 7 |
| C2-1 | 12 |

Even with the major reduction in the number of loose fibers on the surface of the papers superior mechanical properties are maintained versus a control paper of similar average composition but with no layering (Table 6). The low shrinkage at 300°C along with the high tear and tensile properties as compared with the control is especially noteworthy.

**Table 6**

| Calendered Paper Properties | | | |
|---|---|---|---|
| Sample Number | 2-1 | 2-2 | C2-1 |
| Basis Weight, oz/yd² | 4.3 | 4.3 | 4.1 |
| (g/m²) | (145.7) | (145.8) | (139.0) |
| Thickness, mils | 7.5 | 6.7 | 6.8 |
| (mm) | (0.191) | (0.170) | (0.173) |
| Density, g/cc | 0.77 | 0.87 | 0.80 |
| B.S., lb/in MD/CD | 55/30 | 61/39 | 54/33 |
| (N/cm) | (96/53) | (107/68) | (95/58) |
| Eb, % MD/CD | 6/4 | 9/6 | 7/5 |
| Elmendorf Tear, g MD/CD | 695/762 | 421/598 | 504/662 |
| (N) | (6.82/7.48) | (4.13/5.87) | (4.94/6.49) |
| Shrinkage @300°C, % MD/CD | 1/1 | 1/1 | 1/1 |

## Claims

1. A multi-layered calendered aramid paper having a surface suitable for high quality printing characterized in that the paper contains from 40 to 55% by weight of fibrids and comprises a substrate layer which consists essentially of aramid fibrids and floc and one or two surface layers, each bonded to the substrate layer to form a single consolidated sheet, said surface layer(s) comprising from 10 to 67% of the weight of the paper and consisting essentially of from 65 to 90% by weight aramid fibrids and from 10 to 35% by weight aramid floc and wherein the entire surface of the paper is calendered and the sheet has a density of from 0.8 to 1.0 g/cc and a thickness of from 1 to 30 mils (0.0254 to 0.762mm).

2. The paper of Claim 1, wherein said paper comprises two surface layers intimately bonded to opposite sides of said substrate layer.

## Patentansprüche

1. Kalandriertes Mehrschicht-Aramidpapier mit einer Oberfläche, die sich zum Bedrucken in hoher Qualität eignet, dadurch gekennzeichnet, daß das Papier 40 bis 55 Gew.-% Fibride enthält und eine Substratschicht, welche im wesentlichen aus Aramidfibriden und -flockfasern besteht, und eine oder zwei Oberflächenschichten umfaßt, die jeweils an die Substratschicht unter Bildung eines einzelnen verfestigten Flächengebildes gebunden sind, wobei die Oberflächenschicht(en) 10 bis 67 Gew.-% des Papiers ausmacht(en) und im wesentlichen aus 65 bis 90 Gew.-% Aramidfibriden und 10 bis 35 Gew.-% Aramidflockfasern besteht(en), und wobei die gesamte Oberfläche des Papiers kalandriert ist und das Flächengebilde eine Dichte von 0,8 bis 1,0 g/cc und eine Dicke von 1 bis 30 mils (0,0254 bis 0,762 mm) aufweist.

2. Papier nach Anspruch 1, wobei das Papier zwei Oberflächenschichten umfaßt, die innig mit den gegenüberliegenden Seiten der Substratschicht verbunden sind.

## Revendications

1. Papier aramide calandré multicouche avant une surface convenant à une impression de haute qualité, caractérisé en ce que le papier contient de 40 à 55% en poids dc fibrides et comprend une couche de substrat qui consiste essentiellement en floc et fibrides d'aramide et une ou deux couches superficielles, chacune étant liée à la couche de substrat pour former une feuille unique consolidée, cette ou ces couches superficielles formant de 10 à 67% du poids du papier et consistant essentiellement en 65% à 90% en poids de fibrides d'aramide et en 10% à 35% en poids de floc d'aramide et dans lequel la surface totale du papier est calandrée et la feuille obtenue présente une densité de 0,8 à 1.0 g/cm³ et une épaisseur de 0,0254 à 0,762 mm (1 à 30 mils).

2. Papier suivant la revendication 1, ledit papier comprenant deux couches superficielles liées étroitement aux faces opposées de cette couche de substrat.
